

Apr. 3, 1923.

1,450,231

R. F. SALISBURY

METHOD OF MAKING STEAM JACKETED KETTLE OUTLETS

Filed Mar. 20, 1922



WITNESS

*AB Wallace*

INVENTOR

*Robert F. Salisbury*  
By *Winter + Brown*

*Winter + Brown* ATTORNEYS

## UNITED STATES PATENT OFFICE.

ROBERT FLOYD SALISBURY, OF NEW KENSINGTON, PENNSYLVANIA, ASSIGNOR TO  
ALUMINUM COMPANY OF AMERICA, OF PITTSBURGH, PENNSYLVANIA, A CORPO-  
RATION OF PENNSYLVANIA.

## METHOD OF MAKING STEAM-JACKETED KETTLE OUTLETS.

Application filed March 20, 1922. Serial No. 545,390.

To all whom it may concern:

Be it known that I, ROBERT FLOYD SALISBURY, a citizen of the United States, and a resident of New Kensington, in the county of Westmoreland and State of Pennsylvania, have invented a new and useful Improvement in Methods of Making Steam-Jacketed Kettle Outlets, of which the following is a specification.

10 This invention relates to a method of forming a tubular connection between two spaced metallic walls and particularly to an outlet connection for steam-jacketed kettles which must be of such character as to maintain the space between the walls hermetically sealed against comparatively high pressures.

It is the object of the invention to provide a method of forming such an outlet that is 20 simple and easily performed, which will produce a hermetically sealed connection, all joints of which are firmly and durably united, and which will not easily tear away when subjected to subsequent strains. It 25 is a special object to form an outlet of the character referred to in which the walls and the parts forming the same are made of a metal which loses or greatly diminishes in ductility when it becomes heated to a temperature approaching that necessary to effect a weld, or which has a high coefficient 30 of expansion, or both, such as aluminum, and to obviate corrosion adjacent the joints of the finished connection.

35 The method can best be disclosed by illustrating and describing the same as actually performed in connection with a typical device. A steam jacketed kettle of an approved type has, therefore, been selected 40 and the invention as it is carried out in forming the outlet connection thereto will be described.

The single figure of the drawing is a 45 fragmentary view partly in section and partly in elevation showing the finished outlet connection to a steam jacketed kettle formed according to the invention.

The inner and outer shells or walls of the kettle are indicated at 1 and 2, respectively, 50 the same being spaced apart to provide a steam heating chamber therebetween, the lower portion of which is illustrated at 3. The outlet in the embodiment shown is of tubular form adapted to discharge the con-

tents from within the kettle, through a pipe 55 (not shown) threaded to its outer extremity.

If the walls 1 and 2 are made of aluminum, and other metals are used in the portions forming the connection which contact the aluminum parts, that is, if some of the 60 parts of the connections are of aluminum and parts formed of other metals, such as brass, abut the aluminum parts, an electrolytic or other similar action has been found to be set up, causing a pronounced corrosion 65 in and adjacent the joints between the two metals. If all the parts are constructed of the same metal, and the metal is of such character as to lose or greatly diminish in ductility when the same is highly heated, 70 that is to a temperature approaching that necessary to effect a weld, or if such metal possesses a high coefficient of expansion or both, it is extremely difficult to secure a durable hermetically sealed welded joint between the several parts which will effectively withstand the pressures of heating fluids often used, due to the stresses set up 75 between the parts before the portions adjacent the weld have regained their ductility. 80

The invention produces a simple and efficient connection free of corrosion between the parts, and in which the several parts are strongly attached and tightly sealed. In the first place, all the parts are of the same 85 metal thereby eliminating corrosion resulting from the cause above noted, and in the second place, a proper sequence in welding the several joints is followed, thereby overcoming the disadvantages arising from the 90 physical properties of the metal, to be presently described.

The inner shell 1 is flared outwardly 95 around its central aperture 4 to form an annular lip 5 to which one end of the cylindrical tube 6 corresponding in thickness and cross-sectional dimension is welded as indicated at 7, tube 6 being of such length as to project through and for some distance beyond the aperture 8 in the outer shell 2. 100

The space between the exterior of the tube 6 and the edge of aperture 8 is closed by an apertured disk or annulus 9, the curvature of which adapts the same to fit the exterior surface of the shell 2, and the size of its central aperture is such as to form a snug fit around the exterior of the tube 6. After 105 the tube 6 has been welded to the lip 5, the

annulus 9 is positioned as shown in the drawing and is welded to the tube adjacent the line of contact between the disk and tube as indicated at 10. The parts are then allowed to cool, after which the peripheral edge of the disk is welded to the shell 2, as at 11.

Experience has shown that with aluminum or metals having similar characteristics, as above noted if the disk 9 be welded at both lines of contact 10 and 11, either simultaneously or before the disk 9 has been cooled sufficiently to resume its normal dimensions, the welds will be defective and weak due to the stresses set up between the disk and tube and disk and shell, respectively, caused by expansion and contraction of the parts, and the consequent drawing away of the same in conjunction with the lack or diminished ductility in the metal incident to its highly heated condition in the region of the welded joints.

Heretofore, many attempts have been made to weld the outer shell 2 directly to the periphery of the tube 6 but due to the peculiarities of metals of the class named, as above pointed out, the results were very unsatisfactory, a large percentage of the welded joints being defective to a greater or less extent. If, however a disk of suitable proportions is used and the parts are cooled after welding at 10 and before the disk and shell 2 are welded together at 11, a perfect weld and hermetically sealed joint is secured capable of easily withstanding any pressures ordinarily used.

It is well known that more satisfactory welds can be secured provided the parts to be united are heated to substantially the same temperature during the welding process. By employing the present method it is found that the parts welded together can be brought approximately to the same temperature in the region of the welded connection resulting in substantially perfect welds. It is obvious that expansion and contraction of the tube 6 also tends to set up certain stresses, but due to the sequence of operations employed as above described, the same do not tend to rupture the joint 10 due to the fact that the disk 9 is freely suspended during the first welding operation and becomes negligible from a practical standpoint during the welding of the joint 11.

While the applicability of the invention has been described in connection with the use of metal parts, all of which are of aluminum, the walls connected being curved, and the main body of the connection being of tubular form, it is obvious that the invention is equally applicable to metals having similar characteristics and whether the walls be curved, irregular or straight. It is, therefore, not intended to limit the invention

beyond that specifically set forth and defined in the appended claims.

I claim:

1. The method of forming an outlet for steam jacketed kettles comprising spaced metallic walls which consists in hermetically joining a tubular metal body to one of said walls and permitting the same to extend through and beyond an aperture in the other wall, embracing the body with a close fitting apertured disk, welding the disk to the body, cooling the disk, and welding the disk to the second named wall. 70 75

2. The method of forming an outlet for steam jacketed kettles comprising two spaced metallic walls which consists in welding the tubular metal body to one wall, permitting the body to project through an aperture in the other wall, positioning a snug fitting apertured disk over the body, welding the disk to the body, cooling the disk, and welding the disk to the second named wall. 80 85

3. The method of forming an outlet for steam jacketed kettles comprising two spaced metallic walls which consists in welding a tubular metal body to a portion of one wall projecting towards the other wall and permitting the same to extend through an opening in the other wall, embracing the body with a close fitting apertured disk, welding the disk to the body adjacent their line of contact, cooling the disk, and welding the peripheral edge of the disk to the second named wall. 90 95

4. The method of forming an outlet for steam jacketed kettles comprising spaced metallic walls which consists in welding a tubular body so as to surround an aperture in one wall, permitting the body to extend through and beyond an opening in the other wall, embracing the projecting extremity of said body with a close fitting annulus, welding the annulus to the exterior of the body adjacent and throughout their entire line of contact, cooling the annulus, and welding the peripheral edge of the annulus to the second named wall. 100 105 110

5. The method of forming an outlet for steam jacketed kettles comprising two spaced metallic walls which consists in forming an annular lip around an opening in one wall projecting within the space between the walls, welding one end of a cylindrical tube to the lip permitting the opposite end of the tube to extend through and beyond an opening in the other wall, embracing the projecting end of the tube with a close fitting annulus, welding the annulus to the tube adjacent and throughout their line of contact, cooling the annulus, and welding the annulus to the other wall. 115 120 125

6. The method of forming an outlet for steam jacketed kettles comprising spaced metallic walls which consists in forming an annular lip around an opening in one wall 130

- projecting within the space between the walls, welding one end of a cylindrical tube to the lip to form a hermetically sealed joint and permitting the opposite end of the tube 5 to extend through and beyond an opening in the other wall, embracing the projecting end of the tube with a close fitting annulus, welding the annulus to the tube adjacent and throughout their line of contact, cool- 10 ing the annulus, and welding the peripheral edge of the annulus to the exterior of the second named wall.
7. The method of forming an outlet for steam jacketed kettles comprising two spaced 15 walls made of metal possessing a high coefficient of expansion which consists in welding a tubular body of similar metal to one of the walls permitting the same to project through an opening in the other wall, embr- 20 acing the body with a close fitting apertured disk also of the same metal, welding the disk and body adjacent their line of contact, cooling the disk, and welding the disk to the second named wall.
8. The method of forming an outlet for steam jacketed kettles comprising two spaced 25 walls made of metal which loses or greatly diminishes in ductility when highly heated, which consists in welding a tubular body of similar metal to one of the walls permitting the same to project through an opening in the other wall, embr- 30 acing the body with a close fitting apertured disk also of the same metal, welding the disk and body adjacent
- their line of contact, cooling the disk, and 35 welding the disk to the second-named wall.
9. The method of forming an outlet for steam jacketed kettles comprising two spaced walls made of metal possessing a high coeffi- 40 cient of expansion and which loses or greatly diminishes in ductility when highly heated, consisting in welding a tubular body of simi- 45 lar metal to one of the walls permitting the same to project through an opening in the other wall, embracing the body with a close fitting apertured disk also of the same material, welding the disk and body adjacent their line of contact, cooling the disk, and welding the peripheral edge of the disk to the second named wall. 50
10. The method of forming an outlet for steam jacketed kettles comprising two spaced aluminum walls which consists in forming an annular lip around an opening in one wall projecting towards the other wall, weld- 55 ing one end of a cylindrical aluminum tube to the lip permitting the opposite end there- of to project through an opening in the sec- ond named wall, embracing the projecting end of the tube with a close fitting annulus also of aluminum, welding the annulus to the tube, cooling the parts, and welding the annulus to the second named wall. 60

In testimony whereof, I sign my name.  
ROBERT FLOYD SALISBURY.

Witnesses:

Jos. T. WEINZIERL,  
P. B. HETRICK.